

# UNITED STATES PATENT OFFICE.

WILLIAM WHITE, JR., OF PITTSBURG, PENNSYLVANIA.

## MANUFACTURE OF STEEL.

SPECIFICATION forming part of Letters Patent No. 695,256, dated March 11, 1902.

Application filed July 11, 1901. Serial No. 67,901. (No specimens.)

To all whom it may concern:

Be it known that I, WILLIAM WHITE, Jr., a citizen of the United States, residing at Pittsburgh, in the county of Allegheny and State of Pennsylvania, have invented or discovered certain new and useful Improvements in the Manufacture of Steel, of which improvements the following is a specification.

The invention described herein relates to certain improvements in the manufacture of open-hearth steel, and has for its object the shortening of the time required in the elimination of the silicon, carbon, phosphorus, &c., from the metal and a more perfect control of such elimination.

The length of time required for the treatment of metal by the open-hearth method is the principal objection to its practice. Under usual conditions of practice it is impossible to make more than twelve to eighteen heats a week, dependent upon the percentage of silicon, carbon, &c., contained in the metal treated and the extent of elimination required. The long time required in the treatment of the metal in the open-hearth process is due largely to the fact that the eliminations or reductions of the silicon, carbon, &c., are to a large extent successive, being effected at different temperatures—that is to say, the elimination of the silicon occurs at a lower temperature than that of the carbon and ceases almost entirely at the temperature at which the carbon is eliminated most efficiently by reason of the greater affinity between oxygen and carbon at such a high temperature. It has been attempted to employ bessemerized metal in the open-hearth process, the silicon, carbon, &c., being eliminated as far as possible in the converter and the metal transferred to the open hearth for further treatment. This method has not been practically successful as the metal is too hot after treatment in the converter and must be allowed to cool before open-hearth treatment can begin, and, further, in the bessemerizing treatment the temperature is increased so rapidly by the oxidation of the silicon that it passes beyond the desiliconizing temperature before all or the desired percentage of silicon is eliminated, so that the metal when transferred to the open hearth is too high in

silicon, and such excess must be removed in the open hearth.

In the practice of my invention molten metal at a desiliconizing temperature is charged into a converter and blown to effect an elimination of the silicon. In the oxidation out of the silicon from a fifteen-ton charge containing two per cent. silicon between nine and ten million heat units will be developed by the continuation of the blast for ten minutes. The development of this heat unless neutralized would soon raise the metal beyond the desiliconizing temperature—*i. e.*, to a temperature at which the oxygen has greater affinity for carbon than silicon—and that before the silicon has been sufficiently eliminated. Hence I provide for maintaining the metal at a desiliconizing temperature until the carbon lines in the spectrum show that elimination of carbon is actually progressing. A convenient means for preventing an injurious or detrimental increase of temperature by the burning of the silicon consists in forcing steam into the converter with the air. I have found that if in treating a fifteen-ton charge of metal containing two per cent. silicon steam at or about one hundred and twenty-five pounds pressure be forced into the converter through a pipe one and a half inches in diameter the metal can be maintained at a desiliconizing temperature and any desired percentage of silicon removed. As soon as all or the desired percentage of silicon has been removed the metal is transferred to an open-hearth furnace by any suitable means and there treated for the removal of carbon or phosphorus or impurities by any of the usual or known methods.

It will be understood by those skilled in the art that during the latter part of the treatment in the converter the steam may be partially or entirely cut off, so that the temperature of the metal will be increased to or nearly to the point at which carbon is oxidized, so that when charged into the open-hearth furnace decarburization may proceed immediately, and there will not be any delay in heating the bath to the required temperature. As there will not be any material oxidation of the iron in the converter as long as either silicon or carbon is present, the metal will

not be in any way injured by the Bessemer treatment. As the metal is desiliconized rapidly in the converter and as only the carbon or a portion thereof has to be removed in the open-hearth furnace, it is evident that time required required in reducing the pig-iron to steel will be very much shorter than in the ordinary open-hearth treatment and that this shortening of the time will not produce any injurious effects on the metal.

I claim herein as my invention—

1. As an improvement in the art of manufacturing steel, the method herein described which consists in charging molten metal into a converter, blowing air through the metal to remove the silicon, neutralizing the heat developed by the burning of the silicon, transferring the desiliconized metal to an open-hearth furnace and subjecting it to the usual or any desired treatment, substantially as set forth.

2. As an improvement in the art of manu-

facturing steel, the method herein described, which consists in subjecting molten metal to the action of a blast of air for the removal of the silicon; neutralizing the heat developed by the burning of the silicon and finally subjecting the desiliconized metal to treatment in an open-hearth furnace, substantially as set forth.

3. As an improvement in the art of manufacturing steel, the method herein described, which consists in charging molten metal into a converter, forcing air and steam through the metal, transferring the metal when desiliconized to an open-hearth furnace, and treating it therein in the usual or any desired manner, substantially as set forth.

In testimony whereof I have hereunto set my hand.

WILLIAM WHITE, JR.

Witnesses:

DARWIN S. WOLCOTT.

F. E. GAITHER